

1

3,046,130

## PHOTOGRAPHIC MATERIALS CONTAINING A CHEMICAL SENSITIZER

Fritz Dersch and Millet R. De Angelus, Binghamton, N.Y., assignors to General Aniline & Film Corporation, New York, N.Y., a corporation of Delaware  
No Drawing. Filed May 12, 1960, Ser. No. 28,525  
19 Claims. (Cl. 96—66)

This invention relates to photographic materials. More particularly, this invention relates to photographic materials sensitized by means of water soluble heterocyclic compounds which are substituted by a polyoxyalkylene chain.

It is well known that polyalkylene oxides such as polyoxyethylene and polyoxypropylene increase the speed of silver halide emulsions. It has also been observed that condensation products of alkylene oxides with amines, carboxylic acids, alcohols, amides or phenols (made according to U.S. Patents 1,970,578 and 2,213,477) and dicyclohexylol-dialkyl methane (see U.S. Patent 2,240,472) have been used as sensitizers. The polyalkylene oxides or the alkylene oxide condensation products should have a molecular weight of at least 300 and preferably 1,500 to 4,000 or more.

The use of the polyalkylene oxides or alkylene oxide condensation products as sensitizers is limited because of their tendency to increase the formation of fog during storage of the photographic film, especially storage at elevated temperature and high humidity. The use of conventional antifogants is not sufficient to satisfactorily eliminate or minimize fog formation in a film coated with an emulsion containing such products as sensitizers. Special antifogants had to be found for use with such emulsions, and, in this connection, reference is made to U.S. Patents 2,704,716, 2,716,062 and 2,728,666.

It is an object of this invention to provide a novel sensitizer for use with a photographic emulsion or with a photographic developer to greatly increase the speed of the emulsion without materially increasing the fogging tendency thereof, any tendency to fog being eliminated or minimized by the use of conventional antifogants.

A further object of this invention is to provide a photographic film comprising a layer containing a water-soluble polyoxyalkylene derivative of a hydroxy- or mercapto-substituted azole in which the polyoxyalkylene chain replaces the hydrogen atom of the mercapto group.

Other objects and advantages of this invention will appear to those skilled in the art from the detailed description thereof given below.

We have now discovered that water-soluble oxyalkylene and polyoxyalkylene derivatives of 2-mercaptopro-2-hydroxy-substituted azoles, namely, condensation products of alkylene oxide, e.g., ethylene oxide or propylene oxide, epichlorhydrine, trimethylene chlorhydrine or glycerol  $\alpha$ -chlorhydrine with a 2-hydroxy- or 2-mercaptopro-substituted azole, e.g., benzothiazole, benzoxazole, benzimidazole or quinoline, have a remarkable speed increasing effect on silver halide emulsions. Surprisingly, these reaction products, unlike the heretofore used polyoxyalkylenes, do not have the objectionable tendency of increasing the fog of photographic films during storage especially under conditions of high temperature and high humidity. The fogging of photographic film having a coating of a silver halide emulsion and containing the novel sensitizer of our invention may, therefore, be controlled by the use of the conventional antifogants and stabilizers used in the photographic art; and the use of a special type of antifogant to prevent fogging of an emulsion containing conventional polyoxyalkylenes such as those disclosed in U.S. Patents 2,704,716, 2,716,062 and 2,728,666 becomes unnecessary.

The polyoxyalkylene substituted heterocyclic com-

2

pounds contemplated for use herein have the following general formula:



wherein A is a sulfur or oxygen atom, R<sub>1</sub> and R<sub>2</sub> are alkylene groups which may be alike or different and contain at least two, but not more than three atoms, X is a sulfur, oxygen, imino or vinylene (—CH=CH—) group, Z represents the atoms necessary to complete an aromatic ring system of the benzene and naphthalene series and n is an integer between 4 and 40 so as to give the compound a molecular weight of at least 300.

Examples of compounds within the ambit of such formulae are:

2-mercaptop-5-benzothiazole,



2-polyoxyethylenemercaptobenzoxazole



2-polyoxyethylenoxybenzothiazole



2-polyoxyethylenemercaptobenzothiazole



2-polyoxyethylenemercaptoquinoline



2-polyoxyethylenepropyleneoxymercaptopbenzimidazole

These heterocyclic polyoxyalkylene compounds are produced by introducing hydroxy aliphatic ether radicals into 2-hydroxy- or 2-mercaptopo-substituted azoles according to the procedure described in United States Patent 2,642,430. Among the suitable azoles are the following:

2-mercaptopbenzimidazole,

2-mercaptopquinoline,

2-mercaptop-4-methylquinoline,

2-mercaptop-benzoxazole,

2-mercaptop-5-methylbenzoxazole,

2-mercaptop-5-methoxybenzoxazole,

2-mercaptop-4,5-benzobenzoxazole,

2-mercaptopbenzothiazole,

2-mercaptop-5-methyl-benzothiazole,

2-mercaptop-5-methoxy-benzothiazole,

2-mercaptop-5-benzobenzothiazole,

2-hydroxy-4-phenyl benzothiazole,

2-hydroxybenzothiazole,

2-hydroxy-4-methylbenzoxazole,

2-hydroxybenzothiazole,

2-hydroxy-4-methylbenzothiazole and the various analogues and homologues thereof.

The above described heterocyclic compounds are condensed with hydroxy compounds such as ethylene oxide, propylene oxide, epichlorhydrine, trimethylene chlorhydrine, glycerol  $\alpha$ -chlorhydrine, glycol, glycerine, poly-glycerine and the like. In some instances, two or more of these compounds are reacted consecutively with the mercapto- or hydroxy-substituted azole. Alkaline reacting compounds such as sodium or potassium hydroxide or heavy metal salts such as nickel sulfate serve as catalyzing agents.

The increase of effective sensitivity of photographic silver halide emulsions with the polyoxyalkylene derivatives of the 2-mercaptop- or 2-hydroxy-substituted heterocyclics can be obtained in a number of ways. They may be added to an undercoating, to a middle coating, to an overcoating or to a surface coating prior to the coating operation. If desired, they may be added during the actual preparation of the emulsion, either before or after washing of the emulsion.

The speed and sensitivity increasing agents of our invention may be used in various types of photographic emulsions; e.g., nonsensitized emulsions, orthochromatic, panchromatic, and X-ray emulsions. If used with sensitizing dyes, they may be added to the emulsion before or after the dyes are added. Various silver salts may be used as a sensitive element, such as silver bromide, silver iodide, silver chloride or mixed silver halides. These hydroxy-substituted ether or thioether derivatives of heterocyclic compounds may be used in emulsions intended for color photography, e.g., emulsions containing color-forming components. The carrier in the photographic emulsion may be gelatin or other colloids such as collodion, albumen, cellulose derivatives, polyvinyl alcohol or synthetic resins. The emulsion containing our novel sensitizer may be coated on any conventional base, such as paper, glass, cellulose ester such as cellulose acetate, cellulose ethers and others.

The amounts of sensitivity increasing agents used per kilogram of emulsion range from 15 to 500 milligrams per kilogram of liquid emulsion. When expressed in terms of silver halide, the amounts of sensitivity increasing agents range from 25 to 500 milligrams per mole of silver halide.

The sensitivity increasing agents of our invention can also be added to pre-bath solutions or to standard developer solutions. These developer solutions contain, in addition to the speed increasing agent, a developing agent such as metol, hydroquinone 1-phenyl - 3 - pyrazolidone (phenidone); an alkali such as sodium or potassium carbonate; a preservative or anti-oxidant such as sodium sulfite; and an antifoggant such as potassium bromide. The amounts of speed increasing agents used range from 0.3 to 6.0 grams per liter of developer solution.

The following specific examples are given of the manner of producing and using the sensitizers of our invention. It is to be understood, however, that these examples are given by way of illustration and not by way of limitation.

#### Example I



A silver halide emulsion in gelatin containing 4 percent silver iodide and 96 percent silver bromide was prepared in a conventional manner and brought up to its maximum light sensitivity. It was then readied for coating on film base, that is, melted at 40° C.; and the necessary coating finals were added, such as sensitizing dyes, stabilizers and hardeners. A 10 percent aqueous solution of the reaction product of 2-mercaptopbenzimidazole and 6 moles of ethylene oxide was prepared, and 10 cc. of this solution were added to a sample of the above described

emulsion containing about 0.4 mole of silver halide. A sample of the same emulsion, but not containing the speed increasing additive, served as a control. A second control was prepared by adding polyoxyethylene lauryl ether to a third emulsion sample. The so-prepared emulsion samples were coated on a suitable cellulose ester base and dried. Samples of these film coatings were then exposed in a type II-B sensitometer and developed in a developer of the following composition:

|                                     | Grams |
|-------------------------------------|-------|
| Metol (p-methylaminophenol sulfate) | 1.5   |
| Sodium sulfite, anhydrous           | 45.0  |
| Sodium bisulfite                    | 1.0   |
| Hydroquinone                        | 3.0   |
| Sodium carbonate, monohydrated      | 6.8   |
| Potassium bromide                   | 8     |
| Water to make 1.0 liter.            |       |

The developed films were short-stopped, fixed and washed in the conventional manner. The results obtained were as follows:

|                                                                              | Relative speed | Fog            |                               |
|------------------------------------------------------------------------------|----------------|----------------|-------------------------------|
|                                                                              |                | After 12' Dev. | 6 Days' Oven Test and 6' Dev. |
| Quantity of reaction product of 2-mercaptopbenzimidazole and ethylene oxide: |                |                |                               |
| 0                                                                            | 100            | .20            | .14                           |
| 60 milligrams                                                                | 150            | .21            | .14                           |
| 100 milligrams                                                               | 160            | .22            | .14                           |
| Quantity of Polyoxyethylene lauryl ether added:                              |                |                |                               |
| 100 milligrams                                                               | 150            | .28            | .20                           |

The ethylene oxide derivative of 2-mercaptopbenzimidazole which served as a sensitizer was prepared as follows: 50 grams of 2-mercaptopbenzimidazole was mixed with 0.5 gram of potassium hydroxide which had been dissolved in a minimum amount of water; the mass was heated to 130° C.; ethylene oxide was passed through until 6 moles of ethylene oxide had been taken up.

#### Example II



The procedure was the same as in Example I excepting that there was used the reaction product of 2-mercaptopbenzimidazole and trimethylene chlorhydrine which was then condensed with 8 moles of ethylene oxide. The results were similar to those obtained in Example I.

This addition product was prepared as described in Example VI of United States Patent 2,642,430.

60

#### Example III



The procedure was the same as in Example I excepting that there was used the reaction product of 2-mercaptopquinoline and 12 moles of ethylene oxide. The results were similar to those of Example I.

70

The compound was prepared by heating 2-mercaptopquinoline to 200° C. and passing ethylene oxide through the melted mass until the weight increase corresponded to 12 moles of ethylene oxide. A small amount of potassium hydroxide served as the condensation catalyst.

5  
Example IV

The procedure was the same as in Example I excepting that the reaction product of 2-hydroxybenzothiazole and 4 moles of propylene oxide iodide was used. The results were similar to those obtained in Example I.

The compound was prepared by heating under reflux 1 mole of 2-hydroxybenzothiazole and 1 mole of propylene oxide for 1 hour using a small amount of potassium hydroxide. Additional increments of propylene oxide were added while heating and refluxing continued until a total of 4 moles of propylene oxide had been consumed.

## Example V

One kilo of a silver halide emulsion in gelatin containing 4 percent silver iodide and 96 percent silver bromide was coated on film base in a manner known to the art. After the coating was performed, an aqueous gelatin solution containing 20 grams of gelatin per liter and 20 milligrams of the polyoxyethylene derivative of 2-mercaptopbenzimidazole of Example I was coated thereon as an anti-abrasion layer. After drying, film samples were exposed and processed as described in Example I. The samples described exhibited a relative speed of 150 with a fog of .22 as compared with a type coating of the same emulsion having an anti-abrasion layer similar to that described above, but lacking the speed increasing additive and having a speed of 100 and a fog of .20.

## Example VI

Several samples of a conventional photographic film were exposed in a type II-B sensitometer and then divided into two groups. One group of samples was developed for twelve minutes at 68° F. in a standard metol-hydroquinone developer as described in Example I. The other group of samples was developed for the same length of time and at the same temperature as the first group in a metol-hydroquinone developer which had been prepared by adding to 1 liter of the developer described in Example I, 2 grams of the reaction product of ethylene oxide and 2-mercaptopbenzimidazole. It was found that the samples developed in the standard developer had a relative speed of 100 whereas the samples developed in the developer containing the novel sensitivity increasing agent of our invention showed a relative speed of 175 without an increase in fog.

Modifications of the invention will occur to persons skilled in the art. Thus, it is evident that in lieu of the ethylene oxide addition products of the examples, any of the addition products mentioned above may be employed in our invention. We, therefore, do not intend to be limited in the patent granted except as necessitated by the appended claims.

We claim:

1. A light-sensitive silver halide emulsion containing as a sensitizer therefor, a water soluble heterocyclic polyoxyalkylene compound selected from the group consisting of those having the following general formula:



wherein A is a member selected from the group consisting of oxygen and sulfur; R<sub>1</sub> and R<sub>2</sub> are alkylene groups containing from 2 to 3 carbon atoms; X represents the atoms necessary to complete a heterocyclic mononuclear ring and is a member selected from the group consisting of oxygen, sulfur, imino and vinylene; Z represents the

## 6

atoms necessary to complete an aromatic ring system of the benzene and naphthalene series; and n is an integer between 4 and 40.

2. A light-sensitive silver halide emulsion containing as a sensitizer therefor, a compound of the following formula:



wherein n is an integer between 4 and 40.

3. A light-sensitive silver halide emulsion containing as a sensitizer therefor, a compound of the following formula:



wherein n is an integer between 4 and 40.

4. A photographic material comprising a base and a gelatino silver halide emulsion layer containing as a sensitizer therefor, a water soluble heterocyclic polyoxyalkylene compound of the following formula:



wherein A is a member selected from the group consisting of oxygen and sulfur; R<sub>1</sub> and R<sub>2</sub> are alkylene groups containing from 2 to 3 carbon atoms; X represents the atoms necessary to complete a heterocyclic mononuclear ring and is a member selected from the group consisting of oxygen, sulfur, imino, vinylene; and Z represents the atoms necessary to complete an aromatic ring system of the benzene and naphthalene series; and n is an integer between 4 and 40.

5. A photographic material comprising a base and a light-sensitive silver halide emulsion layer containing as a sensitizer therefor, a compound of the following formula:



wherein n is an integer between 4 and 40.

6. A photographic material comprising a base and a light-sensitive silver halide emulsion layer containing as a sensitizer therefor, a compound of the following formula:



wherein n is an integer between 4 and 40.

7. A photographic material comprising a base and a light-sensitive silver halide emulsion layer containing as a sensitizer therefor, a compound of the following formula:



wherein n is an integer between 4 and 40.

8. The process of increasing the sensitivity of a light-sensitive silver halide material comprising a base having a light-sensitive silver halide emulsion thereon which

comprises exposing said emulsion and developing the same in the presence of a water-soluble heterocyclic polyoxyalkylene compound selected from the group consisting of those having the following general formula:



wherein A is a member selected from the group consisting of oxygen and sulfur; R<sub>1</sub> and R<sub>2</sub> are alkylene groups containing from 2 to 3 carbon atoms; X represents the atoms necessary to complete a heterocyclic mononuclear ring and is a member selected from the group consisting of oxygen, sulfur, imino and vinylene; Z represents the atoms necessary to complete an aromatic ring system of the benzene and naphthalene series; and n is an integer between 4 and 40.

9. The process of increasing the sensitivity of a light-sensitive silver halide material comprising a base having a light-sensitive silver halide emulsion thereon, which comprises exposing said emulsion and developing the same in the presence of a compound having the following formula:



wherein n is an integer between 4 and 40.

10. The process of increasing the sensitivity of a light-sensitive silver halide material comprising a base having a light-sensitive silver halide emulsion thereon, which comprises exposing said emulsion and developing the same in the presence of a compound having the following formula:



wherein n is an integer between 4 and 40.

11. The process of increasing the sensitivity of a light-sensitive silver halide material comprising a base having a light-sensitive silver halide emulsion thereon, which comprises exposing said emulsion and developing the same in the presence of a compound having the following formula:



wherein n is an integer between 4 and 40.

12. A photographic developer solution comprising a silver halide developing agent, an alkali, an anti-oxidant and an antifogging agent containing as a speed increasing agent a water-soluble heterocyclic polyoxyalkylene compound selected from the group consisting of those having the following general formula:



wherein A is a member selected from the group consisting of oxygen and sulfur; R<sub>1</sub> and R<sub>2</sub> are alkylene groups containing from 2 to 3 carbon atoms; X represents the atoms necessary to complete a heterocyclic mononuclear ring and is a member selected from the group consisting of oxygen, sulfur, imino and vinylene; Z represents the atoms necessary to complete an aromatic ring system of the benzene and naphthalene series; and n is an integer between 4 and 40.

atoms necessary to complete an aromatic ring system of the benzene and naphthalene series; and n is an integer between 4 and 40.

13. A photographic developer solution comprising a silver halide developing agent, an alkali, an anti-oxidant, an antifogging agent, and containing as a speed increasing agent a compound of the following formula:



15 wherein n is an integer between 4 and 40.

14. A photographic developer solution comprising a silver halide developing agent, an alkali, an anti-oxidant, an antifogging agent, and containing as a speed increasing agent a compound of the following formula:



20 wherein n is an integer between 4 and 40.

15. A photographic developer solution comprising a silver halide developing agent, an alkali, an anti-oxidant, an antifogging agent, and containing as a speed increasing agent a compound of the following formula:



25 wherein n is an integer between 4 and 40.

16. A photographic material comprising a base having a layer of a light-sensitive silver halide emulsion thereon, said silver halide layer being in contiguous contact with another layer comprising a colloidal carrier and a water-soluble heterocyclic polyoxyalkylene compound selected from the group consisting of those having the following general formula:



wherein A is a member selected from the group consisting of oxygen and sulfur; R<sub>1</sub> and R<sub>2</sub> are alkylene groups containing from 2 to 3 carbon atoms; X represents the atoms necessary to complete a heterocyclic mononuclear ring and is a member selected from the group consisting of oxygen, sulfur, imino and vinylene; Z represents the atoms necessary to complete an aromatic ring system of the benzene and naphthalene series and n is an integer between 4 and 40.

17. A photographic material comprising a base having a layer of a light-sensitive silver halide emulsion thereon, said silver halide being in contiguous contact with another layer comprising a colloidal carrier and a compound of the following formula:



70 wherein n is an integer between 4 and 40.

18. A photographic material comprising a base having

a layer of a light-sensitive silver halide emulsion thereon, said silver halide being in contiguous contact with another layer comprising a colloidal carrier and a compound of the following formula:



wherein  $n$  is an integer between 4 and 40.

19. A photographic material comprising a base having a layer of a light-sensitive silver halide emulsion thereon, said silver halide being in contiguous contact with

another layer comprising a colloidal carrier and a compound of the following formula:



wherein  $n$  is an integer between 4 and 40.

References Cited in the file of this patent

UNITED STATES PATENTS

2,944,902 Carroll et al. ----- July 12, 1960